# EUROPEAN PATENT SPECIFICATION

(11) **EP 0 578 642 B1**
(45) Date of publication and mention of the grant of the patent: **02.10.2002**
(21) Application number: 92904376.8
(22) Date of filing: 04.02.1992
(51) Int. Cl.: C10M 127/02, C10N 30/04, C10N 40/25

(54) **LUBRICATING OIL COMPOSITION**
SCHMIERÖLZUSAMMENSETZUNG
COMPOSITION D'HUILE LUBRIFIANTE

(30) Priority: 04.02.1991 AU 442591; 04.11.1991 AU 925991; 13.12.1991 AU 999491; 23.01.1992 AU 53192
(43) Date of publication of application: 19.01.1994
(73) Proprietor: MUNTZ, Pieter Jan Dirk, South Perth, W.A. 6151 (AU)
(72) Inventor: MUNTZ, Pieter Jan Dirk, South Perth, W.A. 6151 (AU)
(74) Representative: Pendlebury, Anthony
(86) International application number: AU9200034
(87) International publication number: WO92013932

(56) References cited:
- EP-A- 0 332 433
- DD-A- 209 846
- DD-A- 280 545
- DE-A- 2 607 614
- GB-A- 1 572 794
- GB-A- 2 224 287
- US-A- 1 966 111
- US-A- 4 023 980
- US-A- 4 737 537
- DERWENT ABSTRACT Accession No. 92299B/51, Class L02; & SU,A,655544 (AS KAZA PETRO NATUR) 9 April 1977 (09.04.77).
- DERWENT ABSTRACT Accession No. 89-118959/16, Class P51; & JP,A,01 065 194 (IDEMITSU KOSAN KK) 10 March 1989 (10.03.89).
- DERWENT ABSTRACT Accession No. 84-240081/39, Class V03; & JP,A,59 142 292 (ALPS ELECTRIC KK) 15 August 1984 (15.08.84).
- DERWENT ABSTRACT Accession No. 84-104339/17, Class H07 L01; & JP,A,59 047 297 (MATSUSHITA ELEC WORKS) 16 March 1984 (16.03.84).
- PATENTS ABSTRACTS OF JAPAN, C-603, page 107; & JP,A,01 048 896 (FURUKAWA ALUM CO LTD) 23 February 1989 (23.02.89).
- PATENTS ABSTRACTS OF JAPAN, C-26, page 152; & JP,A,55 090 590 (MATSUMURA SEKIYU KENKYUSHO K.K.) 9 July 1980 (09.07.80).
- PATENTS ABSTRACTS OF JAPAN, C-84, page 57; & JP,A,56 120 798 (MITSUBISHI DENKI K.K.) 22 September 1981 (22.09.81).

## Description

The present invention relates to lubricating oil compositions.

When two metal surfaces move over each other, considerable heat is evolved due to friction. The function of a lubricant is to separate the two rubbing surfaces by a film thereby greatly reducing the coefficient of friction. If this film fails, the frictional heat produced may melt the surfaces causing them to weld together or seize. When conditions are such that a continuous thick (>0.001 in.) film of lubricant separates the solid surfaces at all points, then frictional resistance is controlled by the viscosity of the lubricant. This is referred to as "hydrodynamic lubrication". Under conditions of high speed or high load, thick lubricant films may be absent or incomplete and lubrication of the parts is effected by layers of adsorbed polar molecules. This situation is referred to as "boundary lubrication". Metal surfaces, which are covered by films of metal oxides, are highly polar and hence are not readily "wetted" by non polar hydrocarbon oils. Used alone, hydrocarbon oils are therefore poor lubricants in these circumstances. Lubricants therefore contain additives which either react with metal surfaces or are adsorbed on the surfaces thereby allowing oil to wet the surface or providing boundary lubrication, thus preventing direct metal to metal contact.

Apart from certain speciality products and synthetic oils, the vast bulk of lubricants are based upon hydrocarbons derived from petroleum.

Crude oils contain a number of broad classes of hydrocarbons, the proportions of which vary greatly from oil to oil.
(a) Branched alkanes. These include iso- and anteiso alkanes, and linear derivates of isoprene such as phytane and pristane and degradation products from molecules such as carotene. These compounds have low melting points and so confer low pour points on lubricating oils. They are also stable to degradation by heat and oxygen and have high viscosity indexes, so this iso-paraffin group is the preferred feedstock for lube oil manufacture.
(b) n-Alkanes. The paraffins have similar properties to the iso-paraffins, except that, due to their higher melting points, they raise the pour point of a lube oil.
(c) Cycloalkanes. The naphthenics contain five-membered and six-membered rings with alkyl side chains. They lower the pour point of an oil but they have a low viscosity index.
(d) Aromatics. These are derivatives of benzene, naphthalene and other fused ring systems with alkyl side chains. This group has a low viscosity index and poor thermal stability.
(e) Sulphur compounds. This group forms a substantial proportion of many crudes, especially those from parts of the Middle East. It has similar properties to aromatics, but are usually even less stable.

In order to prepare a suitable lube oil base stock, a manufacturer will select feeds which have appropriate molecular weight ranges and are rich in the desired classes of hydrocarbons (iso-paraffins), and low in aromatics, ONS compounds, and paraffins so that production costs can be kept low. Crudes such as those from Pennyslvania which are ideal for lube oil manufacture are being depleted, so now most manufacturers use a feed stock mix which is carefully selected to meet the product mix required by the market. Some manufacturers upgrade their feedstock by using a severe hydrogenation/hydrogenolysis process called hydrocracking to remove sulphur, aromatics, and to open rings and crack larger molecules.

The residue from the primary distillation of selected crude oils which are rich in iso-paraffins is distilled at reduced pressure (a few mm of Hg) in the presence of steam. Most usually, three fractions are obtained: two distillate cuts and the residue or bottoms. Typical cuts are shown in the table below.

| **Lubricating Oil Fractions** | | | |
|---|---|---|---|
| Fraction | No. of C atoms | Molecular Weight | Boiling Range °C (Plant conditions) |
| Light (Low viscosity) | 22-36 | 300-500 | 370-500 |
| Medium (medium viscosity) | 29-45 | 400-600 | 450-550 |
| Heavy (high viscosity) | 43 → | 600 → | >500(residue) |

The desired oily alkane material is extracted from the viscous bottoms product from the vacuum tower using liquid propane (high pressure, 65°C) in a propane deasphalting plant. The more polar, high molecular weight polycyclic aromatics are less soluble in liquid propane than are the alkane (paraffin) components and are removed as a hard sludge. Evaporation of the propane leaves the heaviest grade of lubricating oil which is usually referred to as "bright stock".

Each of the lube oil fractions is next treated with a solvent system which selectively removes much of the aromatic and O, N, S material. Phenol and more recently furfural have been widely used in elaborate multistage counter current equipment for this purpose. The immiscible, slightly polar solvent selectively extracts the more polar aromatic material from the hydrocarbon mixture.

n-Alkanes (normal paraffins), which have higher melting points than branched alkanes of similar molecular weight, must be removed to decrease the low temperature viscosity of the lubricating oil. This is accomplished by taking the oil up in a suitable solvent such as a methylethylketone-toluene mixture and chilling 5-10°C below the required pour point. The n-alkanes are precipitated as "slack wax" which is separated by continuous filtration.

The final stage in manufacture of the base stocks is hydrogenation to convert small amounts of dark-coloured unsaturated material into saturated material and to remove sulphur from sulphur compounds present in the oil.

Lubricating oils are finally prepared by blending base stocks to give oil of the desired viscosity range, then introducing many additives to improve the life and performance of the oil.

The chemical composition of lubricating oils derived from crude oil is particularly complex. Normally lubricating oils contain a high proportion of naphthenic or paraffinic compounds. The hydrocarbons comprising a typical lubricating oil may have from 20 to 70 carbon atoms. Usually the hydrocarbons contained in lubricating oil have very few olefinic bonds. However there may be a significant proportion of hydrocarbons exhibiting aromatic unsaturation. A further description of base lubricating oils can be found in an article by D.V. Brock published in "Lubricant Engineering" Volume 43 pages 184-185 March 1987.

Minor improvements in the performance of a lubricating oil can yield significant economic benefits far in excess of the cost of the additive that provides the improved performance. The present invention is based on the discovery that the performance of lubricating oil compositions can be significantly improved by the addition of small amounts of a medium molecular weight paraffin to lubricating oil having typically between about 20 and 70 carbon atoms.

Accordingly the present invention provides a lubricating oil composition comprising a base lubricating oil having typically between about 20 and 70 carbon atoms, characterised by from between 0.1% and 2% by volume of an additive wherein the additive comprises paraffins of medium molecular weight and having between about 10 and 20 carbon atoms, so as to be effective in removing varnish and reducing the coefficient of friction between the surfaces. The medium molecular weight paraffin (MMWP) may comprise from 10 to 20 carbon atoms, from 10 to 19 carbon atoms or from 10 to 17 carbon atoms but preferably it comprises from 10 to 15 carbon atoms. The composition may contain as little as 0.1% by volume of MMWP for an improvement in performance to be observed. Preferably however the engine oil composition of the present invention contains from 0.5% to 1% by volume of a MMWP. Best results have been obtained with about 0.6% by volume MMWP.

MMWP's are normally derived from the processing of crude oils. Normally they are produced during the initial atmospheric distillation of a crude oil and are characterised as hydrocarbons having a boiling point in the range from 150 to 335°C.

The compositions of the present invention may be prepared as compositions ready for use or as concentrates for premixing or mixing in situ e.g. in the sump of an engine. Concentrates may contain as much as 25% of the MMWP. The effective amount of MMWP required depends on the ultimate purpose for its inclusion and may also depend upon the additive selected.

A MMWP of particular interest is one known as "Shellsol T". Shellsol T is characterised as a solvent having the following properties-:

| Property | Test Method | Unit | Specification | Typical Value |
|---|---|---|---|---|
| Distillation | ASTM D1078 | °C | | |
| Ranges, IBP | | | 180 min | 180.2 |
| DP | | | 205 max | 202.5 |
| Flash Point | IP 170 | °C | - | 57.5 |
| Aniline Point | ASTM D611 | °C | 78-83 | 80 |
| Density @ 15°C | ASTM D1298 | kg/ litre | 0.765-0.775 | 0.769 |
| Composition | | %m | | |
| Paraffins | | | | >99.8 |
| Naphthenes | | | | <0.1 |
| Aromatics | | | | <0.1 |

Other products of particular interest are those from the Shellsol series as well as Shell P874, Shell P878 and Ondina Oil 15. Shell P874 and P878 are technical white oils comprising a mixture of paraffins and naphthenes.

Paraffins of medium molecular weight include dodecane, hexadecane, octadecane and cosane.

The lubricating oil compositions of the present invention are based on lubricating oil compositions that are normally commercially available. These compositions may include various additives such as dispersants, detergents, oxidation inhibitors, foam inhibitors, pour point depressants and viscosity improvers. A discussion of the function and formulation of lubricating oil compositions can be found in the "Handbook of Lubrication" Theory and Practice of Tribology Volume 1 edited by E. Richard Booser and published by CRC Press in 1983.

International Patent Application No. PCT/US89/05467, published as WO-A-9007565 discloses lubricating oil compositions containing minute quantities of kerosene, the purpose of which is to carry silicone antifoam formulations into solution in a lubricating oil composition. However the quantities of medium molecular weight paraffins contained in the composition would be insufficient to be effective in the performance of the present invention. Normally the MMWP needs to comprise at least 0.1% to 0.5% by volume of the lubricating oil composition to be effective. Furthermore kerosenes frequently contain substantial proportions of aromatics which may negate the effect of the medium molecular weight paraffin.

The oils of the present invention provide a number of significant advantages over the existing formulations. These include the following.
1. A noticeable reduction in varnishing;
2. A reduction in sludging;
3. Reduced production of harmful chemical by-products such as acids;
4. Improved seal life particularly seals in gear boxes, differentials and engines;
5. Reduced glazing especially when used in the preferred range;
6. Extended life of the oil; and
7. Reduced coefficient of friction of surfaces to which it is applied.

The present invention also includes within its scope methods for any one or more of the following:
a. reducing varnishing in an engine;
b. reducing sludging in an engine;
c. reducing the production of harmful chemical by-products in an engine;
d. improving seal life in an engine; and
e. reducing glazing in an engine by incorporating an effective amount of a medium molecular weight paraffin into a lubricating oil having typically between about 20 and 70 carbon atoms used in the engine.

Benefits provided by the present invention are illustrated by the accompanying comparative examples.

### Example 1

The performance of the compositions of the present invention was compared with the performance of the compositions without the additive of the present invention using a pin on ball testing machine. The pin on ball testing machine comprises an electric motor driving a single shaft through a set of pulleys. A rotatable disc having a diameter of approximately 4cm is attached to the shaft and is rotated at a speed of 1200 - 1500 rpm. A separate shaft is pivoted at one end of the apparatus so that a hardened steel bearing element can be applied to the rotating disc. A torque wrench type configuration fitted to the pivoted shaft is used to determine the load applied to the rotating disc by the hardened steel bearing element.

Lubricant under test was applied to the bearing surface by splashing lubricant from a bath held at a base of the rotating disc. At all times during the test a continuous film of lubricant was in contact with the bearing.

A series of seven oil samples was tested with the apparatus both with and without the addition of the additive. Samples including the additive contained additive in the ratio of 1:80 additive to base lubricating oil composition.

The test procedure was as follows. With the disc rotating, a piece of coarse wet and dry emery paper was used to smooth any imperfections and score marks from the rotating disc prior to test. The bearing was moved to ensure a fresh unmarked surface was available for contact with the rotating disc. Prepared samples were poured into an oil bath containing approximately 20 to 40 mls and held in close contact at the base of the rotating disc which picked oil up and carried it across the bearing surface. The bearing fixed to the pivoted shaft was lowered onto the rotating lubricated disc and allowed to settle in. A continuous load was manually applied to the handle of the pivoted shaft. The load was maintained and gradually increased until the bearing surfaces began to squeal. At the point when squealing commenced, the torque applied was measured in ft.lb units. The results are set out in Table 1.

**TABLE 1**

| **RESULTS FOR OIL ADDITIVE ASSESSMENT** | | | |
|---|---|---|---|
| **Sample** | | **Applied Torque, ft.lb** | |
| | | **Without Additive** | **With Additive** |
| 1. | Shell XMO | 80-100 | 150-160 |
| 2. | Shell Marine Oil | 125 | 160 |
| 3. | BP Engine Oil | 80-110 | 140-150 |
| 4. | BP Gear Oil | 70 | 140 |
| 5. | BP Grease | 130 | 160 |
| 6. | Caltex CXT | 50 | 150 |
| 7. | Esso Tiger | 80 | 150 |

The additive used in this experiment was "Youngs 303" which is a lubricating oil used in cleaning guns. Gas chromatographic analysis of Youngs 303 revealed that it is a mixture of a lubricating oil and another hydrocarbon fraction of slightly higher boiling point than kerosene. The kerosene like fraction had major components of carbon chain length 11 to 13. The kerosene like fraction comprised approximately 50% of the "Youngs 303".

The results demonstrate that the oil additive provides enhanced performance under the harsh boundary lubrication conditions utilised.

### Example 2

The performance of the lubricating oil compositions of the present invention were tested against a base lubricating oil composition in a V8 Caterpillar engine (Model 3408) of 450 horsepower. The results of the test are set out in Table 2. The additive used was Shellsol T in the ratio of 1:160 by volume.

**TABLE 2**

| Test Results V8 CAT Engine | | | | | | | |
|---|---|---|---|---|---|---|---|
| **Test I** | | | | **Test II (with additive)** | | | |
| Time -Mins | Burn Rate/ Hr | Horse Power | R.P.M. | Time -Mins | Burn Rate/ Hr | Horse Power | R.P.M. |
| 5 | 61.7 | 221 | 2183 | 5 | 61.3 | 222 | 2184 |
| 10 | 61.7 | 221 | 2183 | 10 | 61.3 | 222 | 2184 |
| 15 | 61.7 | 221 | 2183 | 15 | 61.3 | 222 | 2184 |
| 20 | 61.7 | 221 | 2183 | 20 | 61.3 | 222 | 2184 |

The results of the test demonstrate that the lubricating oil composition of the present invention increases the power output of the motor and increases fuel efficiency.

### Example 3

A test using a BP lubricating oil as a base was performed on a Holden V8 engine. The additive used was Shellsol T in the ratio 1:160. The results are illustrated in Table 3.

**TABLE 3**

| Holden 253 V8 Using B.P. Oil. | | | |
|---|---|---|---|
| WITHOUT ADDITIVE | | WITH ADDITIVE | |
| L/IDLE | 650 | 775 | 775 |
| H/IDLE | - | - | - |
| H/P | - | - | - |
| TORQUE | 110 | 110 | - |
| W/TEMP | 85 | 95 | 85 |
| OIL/TEMP | - | - | - |
| OIL/PRESS | 120 | 100 | - |
| E/VACUUM | - | - | - |

The dynamometer consistently indicated that the lubricating oil compositions of the present invention resulted in an idle speed that was consistently 125 rpm greater than that for the base lubricating oil.

### Example 4

The lubricating oil composition of the present invention was compared with a base lubricating oil over a range of engine speeds. The additive used was Shellsol T in the ratio 1:160. The engine used was a Caterpillar (Model 3406) six cylinder 400 horsepower engine. The results of the test are shown in Tables 4 and 5. Table 4 illustrates the performance of the engine using the base lubricating oil composition and Table 5 illustrates the performance of the same engine using a lubricating oil composition of the present invention.

**TABLE 4**

| Specifications | | | | | | Test Figures | | |
|---|---|---|---|---|---|---|---|---|
| | | | | | | Without Additive | | |
| Low Idle R.P.M. | | | | 750 | | 758 | | |
| High Idle R.P.M. | | | | 2280 | | 2307 | | |
| Full Load R.P.M. | | | | 2100 | | 2100 | | |
| Rack Setting | | | | 1.15 | | | | |
| Boost Pressure | | | | 33 " | | | | |
| B.S.F.C. | | | | .357 | | | | |
| H.P. Setting | | | | 347 | | | | |
| Lube Oil Pressure at High Idle | | | | | | | | |
| Lube Oil Pressure at Low Idle | | | | | | | | |

| RPM | H.P. | GPH FUEL RATIO | BOOST | EXHAUST TEMP. | FUEL PRESS | WATER TEMP. | OIL TEMP. | OIL PRES |
|---|---|---|---|---|---|---|---|---|
| 2300 | 9 | | 8 | 333 | 230 | 89.3 | 100.9 | 445 |
| 2200 | 223 | | 26 | 365 | 220 | 88.9 | 100.9 | 420 |
| *2100 | 315 | | 45 | 401 | 220 | 89.7 | 100.3 | 415 |
| 2000 | 326 | | 44 | 381 | 220 | 90.2 | 100.1 | 410 |
| 1900 | 322 | | 43 | 377 | 220 | 90.1 | 100.1 | 405 |
| 1800 | 320 | | 43 | 377 | 220 | 89.4 | 99.6 | 400 |
| 1700 | 315 | | 41 | 385 | 220 | 89.6 | 98.6 | 400 |
| 1600 | 309 | | 30 | 401 | 220 | 90.6 | 98.7 | 400 |
| 1500 | 297 | | 27 | 423 | 220 | 90.6 | 99.2 | 400 |
| 1400 | 287 | | 25 | 456 | 220 | 89.7 | 98.5 | 395 |

**TABLE 5**

| Specifications | | | | | | Test Figures | | |
|---|---|---|---|---|---|---|---|---|
| | | | | | | With Additive | | |
| Low Idle R.P.M. | | | | 750 | | 772 | | |
| High Idle R.P.M. | | | | 2280 | | 2304 | | |
| Full Load R.P.M. | | | | 2100 | | 2100 | | |
| Rack Setting | | | | | | | | |
| Boost Pressure | | | | | | | | |
| B.S.F.C. | | | | | | | | |
| H.P. Setting | | | | | | | | |
| Lube Oil Pressure at High Idle | | | | | | | | |
| Lube Oil Pressure at Low Idle | | | | | | | | |

| RPM | H.P. | GPH FUEL RATIO | BOOST | EXHAUST TEMP. | FUEL PRESS | WATER TEMP. | OIL TEMP. | OIL PRES |
|---|---|---|---|---|---|---|---|---|
| *2309 | 38 | | 6 | 292 | 230 | 88.0 | 94.9 | 450 |
| *2200 | 231 | | 24 | 334 | 220 | 89.5 | 96.9 | 440 |
| *2100 | 317 | | 45 | 404 | 220 | 90.6 | 100.3 | 420 |
| 2000 | 326 | | 44 | 398 | 220 | 90.0 | 99.5 | 410 |
| 1900 | 322 | | 43 | 390 | 220 | 89.4 | 99.7 | 400 |
| 1800 | 320 | | 41 | 386 | 220 | 89.9 | 99.8 | 400 |
| *1700 | 318 | | 40 | 394 | 220 | 88.9 | 98.7 | 400 |
| *1600 | 310 | | 30 | 410 | 220 | 89.5 | 98.9 | 400 |
| *1500 | 299 | | 26 | 440 | 220 | 88.7 | 98.2 | 400 |
| 1400 | 284 | | 25 | 467 | 220 | 88.9 | 97.2 | 390 |

The results illustrate that the lubricating oil composition of the present invention produces an increase in power output of 2 to 3 horsepower at low revs and at full load.

### Example 5

Engine Test illustrating anti-varnish benefits:

When added to a 4 litre 6 cylinder engine, which had done over 130,000 kms, and which was beginning to "breathe" noticeably - due to "varnishing", and after approximately 4,000 kms running with an oil change after 2,000 kms with additive, all "breathing" ceased, as observed with the naked eye. The additive used was Shell Sol T in the ratio of 1:160. Combustion was noticeably steadier and more even.

The same experiment was performed with another engine of similar age, and the same results were achieved.

Oil leaks from each of the motors were also reduced and in particular around the crankshaft protrusions.

With the additive included in further oil changes - the result of "no breathing" was continued indefinitely, with the benefit of cleaner oil, next to no oil burning and better running.

Of course along with this other benefits were observed such as improved fuel efficiency, increased engine performance and reduced engine wear.

## Claims

1. A method of reducing varnishing and improving lubrication in mechanical systems selected from the group consisting of internal combustion engines, gear boxes, and differentials which method comprises the step of lubricating the engine, gear box or differential with a lubricating oil composition wherein:
(a) the composition comprises a base lubricating oil having typically from 20 to 70 carbon atoms; and
(b) the composition is **characterised by** from 0.1% to 2% by volume of medium molecular weight paraffin comprising from 10 to 20 carbon atoms;
so as to be effective in removing varnish and reducing the coefficient of friction between surfaces to which it is applied.

2. A method according to claim 1 wherein the medium molecular weight paraffin comprises from 10 to 19 carbon atoms.

3. A method according to claim 2 wherein the medium molecular weight paraffin comprises from 10 to 17 carbon atoms.

4. A method according to claim 3 wherein the medium molecular weight paraffin comprises from 10 to 15 carbon atoms.

5. A method according to any one of claims 1 to 4 wherein the medium molecular weight paraffin is present in proportion from 0.5 to 1.0% by volume.

6. A method according to claim 5 wherein the medium molecular weight paraffin is present in proportion of about 0.6% by volume.

7. A method according to any one of the preceding claims wherein the lubricating oil composition further comprises an additive which additive comprises the medium molecular weight paraffin.

8. A method according to claim 7 wherein the additive comprises a paraffins carbon percentage of greater than 99.8%, a napthenes percentage of less than 0.1% and an aromatic carbon percentage of less than 0.1%, has a flash point of approximately 57.5°C, an aniline point of approximately 78 to 83°C and a density of approximately 0.765 to 0.775 kg/l.

9. A method according to claim 7 wherein the additive also comprises napthenes.

10. A method according to claim 9 wherein in the additive, the paraffins and the napthenes carbon percentages according to the American Society for Testing Materials (ASTM) test method D2140, are approximately 58% and 42% respectively.

11. A method according to claim 10 wherein the additive has a flash point of approximately 106°C, an aniline point of approximately 82°C and a density of approximately 0.807kg/l.

12. A method according to claim 9 wherein in the additive, the paraffins and the napthenes carbon percentages according to the American Society for Testing Materials (ASTM) test method D2140 are approximately 79 and 21% respectively.

13. A method according to claim 12 wherein the additive has a flash point of approximately 146°C, an aniline point of approximately 97°C, and a density of approximately 0.799kg/l.

14. A method according to any one of claims 7 to 13 wherein the additive is present in proportion of 1.25% by volume.

15. A method according to any one of the preceding claims which method further comprises the steps of:
(a) providing a lubricating oil composition comprising the base lubricating oil having typically between 20 and 70 carbon atoms; and
(b) adding the medium molecular weight paraffin to the lubricating oil composition in an amount of from 0.1 to 2.0% by volume of the lubricating oil composition.

16. A lubricating oil composition suitable for use in a method according to any one of claims 5 to 14.

17. Use of a lubricating oil composition in a method of reducing varnishing and improving lubrication in mechanical systems selected from the group consisting of internal combustion engines, gear boxes and differentials wherein:
(a) the lubricating oil composition comprises a base lubricating oil having typically from 20 to 70 carbon atoms; and
(b) the lubricating oil composition is **characterised by** from 0.1% to 2% by volume of a medium molecular weight paraffin comprising from 10 to 20 carbon atoms;
so as to be effective in removing varnish and reducing the coefficient of friction between surfaces to which it is applied.

18. Use according to claim 17 wherein the medium molecular weight paraffin comprises from 10 to 19 carbon atoms.

19. Use according to claim 18 wherein the medium molecular weight paraffin comprises from 10 to 17 carbon atoms.

20. Use according to claim 19 wherein the medium molecular weight paraffin comprises from 10 to 15 carbon atoms.

21. Use according to any one of claims 17 to 20 wherein the lubricating oil composition is as defined in claim 15.

22. A grease composition comprising a thickener and a lubricating oil composition suitable for use according to any one of claims 17 to 21.

23. A grease composition according to claim 22 wherein the thickener comprises a metallic soap.

## Patentansprüche

1. Verfahren zur Reduzierung der Lackbildung und Verbesserung der Schmierung in mechanischen Systemen, ausgewählt aus der Gruppe, bestehend aus Verbrennungsmotoren, Schaltgetrieben und Differentialgetrieben, welches Verfahren den Schritt des Schmierens des Motors, Schaltgetriebes oder Differentialgetriebes mit einer Schmierölzusammensetzung umfasst, wobei:
(a) die Zusammenfassung ein Grundschmieröl mit typischerweise 20 bis 70 Kohlenstoffatomen umfasst; und
(b) die Zusammenfassung **gekennzeichnet ist durch** 0,1 bis 2 Vol.% Paraffin von mittlerer Molekülmasse, umfassend 10 bis 20 Kohlenstoffatome;
um bei der Entfernung von Lack und der Verringerung des Reibungskoeffizienten zwischen Flächen, auf die sie aufgetragen wird, wirksam zu sein.

2. Verfahren gemäß Anspruch 1, wobei das Paraffin von mittlerer Molekülmasse 10 bis 19 Kohlenstoffatome umfasst.

3. Verfahren gemäß Anspruch 2, wobei das Paraffin von mittlerer Molekülmasse 10 bis 17 Kohlenstoffatome umfasst.

4. Verfahren gemäß Anspruch 3, wobei das Paraffin von mittlerer Molekülmasse 10 bis 15 Kohlenstoffatome umfasst.

5. Verfahren gemäß einem der Ansprüche 1 bis 4, wobei das Paraffin von mittlerer Molekülmasse im Ausmaß von 0,5 bis 1,0 Vol.% vorhanden ist.

6. Verfahren gemäß Anspruch 5, wobei das Paraffin von mittlerer Molekülmasse im Ausmaß von etwa 0,6 Vol.% vorhanden ist.

7. Verfahren gemäß einem der vorhergehenden Ansprüche, wobei die Schmierölzusammensetzung weiters einen Zusatz umfasst, welcher Zusatz das Paraffin von mittlerer Molekülmasse umfasst.

8. Verfahren gemäß Anspruch 7, wobei der Zusatz einen Prozentsatz an Paraffin-Kohlenstoff von mehr als 99,8%, einen Prozentsatz an Naphthenen von weniger als 0,1% und einen Prozentsatz an aromatischem Kohlenstoff von weniger als 0,1% umfasst, einen Flammpunkt von etwa 57,5°C, einen Anilinpunkt von etwa 78 bis 83°C und eine Dichte von etwa 0,765 bis 0,775 kg/l besitzt.

9. Verfahren gemäß Anspruch 7, wobei der Zusatz auch Naphthene umfasst.

10. Verfahren gemäß Anspruch 9, wobei die Prozentsätze an Paraffin- und Naphthen-Kohlenstoff im Zusatz gemäß dem Testverfahren D2140 der American Society for Testing Materials (ASTM) etwa 58% bzw. 42% betragen.

11. Verfahren gemäß Anspruch 10, wobei der Zusatz einen Flammpunkt von etwa 106°C, einen Anilinpunkt von etwa 82°C und eine Dichte von etwa 0,807 kg/l besitzt.

12. Verfahren gemäß Anspruch 9, wobei die Prozentsätze an Paraffin- und Naphthen-Kohlenstoff im Zusatz gemäß dem Testverfahren D2140 der American Society for Testing Materials (ASTM) etwa 79% bzw. 21% betragen.

13. Verfahren gemäß Anspruch 12, wobei der Zusatz einen Flammpunkt von etwa 146°C, einen Anilinpunkt von etwa 97°C und eine Dichte von etwa 0,799 kg/l besitzt.

14. Verfahren gemäß einem der Ansprüche 7 bis 13, wobei der Zusatz im Ausmaß von 1,25 Vol.% vorhanden ist.

15. Verfahren gemäß einem der vorhergehenden Ansprüche, welches Verfahren weiters folgende Schritte umfasst:
(a) Bereitstellen einer Schmierölzusammensetzung, umfassend das Grundschmieröl mit typischerweise zwischen 20 und 70 Kohlenstoffatomen; und
(b) Zugabe des Paraffins von mittlerer Molekülmasse zur Schmierölzusammensetzung in einer Menge von 0,1 bis 2,0 Vol.% der Schmierölzusammensetzung.

16. Schmierölzusammensetzung, die zur Verwendung in einem Verfahren gemäß einem der Ansprüche 5 bis 14 geeignet ist.

17. Verwendung einer Schmierölzusammensetzung in einem Verfahren zur Reduzierung der Lackbildung und Verbesserung der Schmierung in mechanischen Systemen, ausgewählt aus der Gruppe, bestehend aus Verbrennungsmotoren, Schaltgetrieben und Differentialgetrieben, wobei:
(a) die Schmierölzusammensetzung ein Grundschmieröl mit typischerweise 20 bis 70 Kohlenstoffatomen umfasst; und
(b) die Schmierölzusammensetzung **gekennzeichnet ist durch** 0,1 bis 2 Vol.% Paraffin von mittlerer Molekülmasse, umfassend 10 bis 20 Kohlenstoffatome;
um bei der Entfernung von Lack und der Verringerung des Reibungskoeffizienten zwischen Flächen, auf die sie aufgetragen wird, wirksam zu sein.

18. Verwendung gemäß Anspruch 17, wobei das Paraffin von mittlerer Molekülmasse 10 bis 19 Kohlenstoffatome umfasst.

19. Verwendung gemäß Anspruch 18, wobei das Paraffin von mittlerer Molekülmasse 10 bis 17 Kohlenstoffatome umfasst.

20. Verwendung gemäß Anspruch 19, wobei das Paraffin von mittlerer Molekülmasse 10 bis 15 Kohlenstoffatome umfasst.

21. Verwendung gemäß einem der Ansprüche 17 bis 20, wobei die Schmierölzusammensetzung so ist wie in Anspruch 15 definiert.

22. Schmiermittelzusammensetzung, umfassend ein Verdickungsmittel und eine Schmierölzusammensetzung, die zur Verwendung gemäß einem der Ansprüche 17 bis 21 geeignet ist.

23. Schmiermittelzusammensetzung gemäß Anspruch 22, wobei das Verdickungsmittel eine Metallseife umfasst.

## Revendications

1. Procédé pour réduire le dépôt de gomme et améliorer la lubrification dans des systèmes mécaniques choisis dans le groupe consistant en des moteurs à combustion interne, des boîtes de vitesse et des différentiels, procédé qui comprend l'étape consistant à lubrifier le moteur, la boîte de vitesse ou le différentiel avec une composition d'huile lubrifiante, dans lequel :
(a) la composition comprend une huile lubrifiante de base ayant habituellement 20 à 70 atomes de carbone ; et
(b) la composition est **caractérisée par** une quantité de 0,1 % à 2 % en volume d'une paraffine de poids moléculaire moyen comprenant 10 à 20 atomes de carbone ;
de manière à être efficace dans l'élimination de la gomme et la réduction du coefficient de frottement entre les surfaces auxquelles elle est appliquée.

2. Procédé suivant la revendication 1, dans lequel la paraffine de poids moléculaire moyen comprend 10 à 19 atomes de carbone.

3. Procédé suivant la revendication 2, dans lequel la paraffine de poids moléculaire moyen comprend 10 à 17 atomes de carbone.

4. Procédé suivant la revendication 3, dans lequel la paraffine de poids moléculaire moyen comprend 10 à 15 atomes de carbone.

5. Procédé suivant l'une quelconque des revendications 1 à 4, dans lequel la paraffine de poids moléculaire moyen est présente en une proportion de 0,5 à 1,0 % en volume.

6. Procédé suivant la revendication 5, dans lequel la paraffine de poids moléculaire moyen est présente en une proportion d'environ 0,6 % en volume.

7. Procédé suivant l'une quelconque des revendications précédentes, dans lequel la composition d'huile lubrifiante comprend en outre un additif, additif qui comprend la paraffine de poids moléculaire moyen.

8. Procédé suivant la revendication 7, dans lequel l'additif comprend un pourcentage de carbone paraffinique supérieur à 99,8 %, un pourcentage de naphtènes inférieur à 0,1 % et un pourcentage de carbone aromatique inférieur à 0,1 %, a un point d'éclair d'approximativement 57,5°C, un point d'aniline d'approximativement 78 à 83°C et une masse volumique d'approximativement 0,765 à 0,775 kg/l.

9. Procédé suivant la revendication 7, dans lequel l'additif comprend également des naphtènes.

10. Procédé suivant la revendication 9, dans lequel, dans l'additif, les pourcentages de carbone de paraffines et de naphtènes suivant la méthode d'essai D2140 de l'American Society for Testing Materials (ASTM) sont, respectivement, égaux à approximativement 58 % et 42 %.

11. Procédé suivant la revendication 10, dans lequel l'additif a un point d'éclair d'approximativement 106°C, un point d'aniline d'approximativement 82°C et une masse volumique d'approximativement 0,807 kg/l.

12. Procédé suivant la revendication 9, dans lequel, dans l'additif, les pourcentages de carbone des paraffines et naphtènes suivant la méthode d'essai D2140 de l'American Society for Testing Materials (ASTM) sont, respectivement, égaux à approximativement 79 et 21 %.

13. Procédé suivant la revendication 12, dans lequel l'additif a un point d'éclair d'approximativement 146°C, un point d'aniline d'approximativement 97°C et une masse volumique d'approximativement 0,799 kg/l.

14. Procédé suivant l'une quelconque des revendications 7 à 13, dans lequel l'additif est présent en une proportion de 1,25 % en volume.

15. Procédé suivant l'une quelconque des revendications précédentes, procédé qui comprend en outre les étapes consistant :
(a) à prendre une composition d'huile lubrifiante comprenant l'huile lubrifiante de base ayant habituellement 20 à 70 atomes de carbone ; et
(b) à ajouter la paraffine de poids moléculaire moyen à la composition d'huile lubrifiante en une quantité de 0,1 à 2,0 % en volume de la composition d'huile lubrifiante.

16. Composition d'huile lubrifiante apte à l'utilisation dans un procédé suivant l'une quelconque des revendications 5 à 14.

17. Utilisation d'une composition d'huile lubrifiante dans un procédé pour réduire le dépôt de gomme et améliorer la lubrification dans des systèmes mécaniques choisis dans le groupe consistant en des moteurs à combustion interne, des boîtes de vitesse et des différentiels, dans laquelle :
(a) la composition d'huile lubrifiante comprend une huile lubrifiante de base ayant habituellement 20 à 70 atomes de carbone ; et
(b) la composition d'huile lubrifiante est **caractérisée par** la présence de 0,1 % à 2 % en volume d'une paraffine de poids moléculaire moyen comprenant 10 à 20 atomes de carbone ;
de manière à être efficace dans l'élimination de la gomme et la réduction du coefficient de frottement entre les surfaces auxquelles elle est appliquée.

18. Utilisation suivant la revendication 17, dans laquelle la paraffine de poids moléculaire moyen comprend 10 à 19 atomes de carbone.

19. Utilisation suivant la revendication 18, dans laquelle la paraffine de poids moléculaire moyen comprend 10 à 17 atomes de carbone.

20. Utilisation suivant la revendication 19, dans laquelle la paraffine de poids moléculaire moyen comprend 10 à 15 atomes de carbone.

21. Utilisation suivant l'une quelconque des revendications 17 à 20, dans laquelle la composition d'huile lubrifiante répond à la définition suivant la revendication 15.

22. Composition de graisse comprenant un épaississant et une composition d'huile lubrifiante apte à l'utilisation suivant l'une quelconque des revendications 17 à 21.

23. Composition de graisse suivant la revendication 22, dans laquelle l'épaississant comprend un savon métallique.
